

## UNITED STATES PATENT OFFICE

MAX DIEPOLD, OF MOSBACH/BADEN, GERMANY

## PROCESS FOR TREATING WHALE BONE BRISTLES

No Drawing. Application filed June 28, 1929, Serial No. 374,614, and in Great Britain and Czechoslovakia February 4, 1929.

This invention is directed to a process for treating whalebone bristles to prevent their deterioration on exposure to moisture.

The practice of using whalebone bristles as a substitute for the ordinary plant fiber bristles in brooms and the like is well known, the commercial advantage residing in the comparatively longer life of the whalebone bristles. Such whalebone bristles, however, suffer a disadvantage as compared with the plant fiber bristles under those conditions where the broom or other similar object is used in places where it is more or less exposed to moisture. Whalebone is particularly receptive to moisture and the absorbence of such moisture by the whalebone breaks down the rigidity of the latter and the bristles become so soft as to be useless for brushing or sweeping purposes.

The primary object of the present invention is a process involving the treatment of whalebone bristles by impregnating such bristles with a specially prepared varnish which is of particular character in that it will not become brittle on drying.

A particular varnish which may be admirably used in connection with the process is made by introducing into methyl alcohol, pinic acid resin and silvic acid and resin, and following this combination vesuvin is added. The resin referred to is rosin or colophony.

The whalebone bristles are treated by being saturated in this varnish or lacquer, and following the saturation and drying of the bristles, they are non-receptive to ordinary moisture and hence articles employing such bristles may take the full advantage of the additional wearing qualities of the whalebone bristles over the plant fiber bristles no matter whether the articles are exposed to moisture or not. The lacquer varnish does not become brittle and therefore the whalebone bristles, when saturated with the varnish, do not lose their inherent flexibility to any appreciable extent.

The process involves the provision of a particular varnish or lac for the saturation of whalebone bristles, with the requirement that such varnish or lac be of a character

to avoid a hardening or rigidity of the whalebone bristles when dry, while at the same time protecting the whalebone against the absorption of moisture.

What is claimed to be new is:

A process for the treatment of whalebone bristles consisting in impregnating said bristles against the absorption of moisture through saturation with a varnish consisting of pinic acid resin, silvic acid and resin, and a vehicle of methyl alcohol, with the addition of vesuvin.

In testimony whereof I affix my signature.

MAX DIEPOLD.

55

60

65

70

75

85

90

95

100